

# UNITED STATES PATENT OFFICE.

OTTO SCHALLER, OF SÜDENDE, NEAR BERLIN, GERMANY, ASSIGNOR TO FIRM: JULIUS  
PINTSCH AKT.-GES., OF BERLIN, GERMANY.

## HOLDER FOR THE GLOWERS OF TUNGSTEN LAMPS.

1,400,005.

Specification of Letters Patent. Patented Dec. 13, 1921.

No Drawing.

Application filed October 27, 1916. Serial No. 128,100.

(GRANTED UNDER THE PROVISIONS OF THE ACT OF MARCH 3, 1921, 41 STAT. L., 1313.)

*To all whom it may concern:*

Be it known that I, Otto Schaller, a subject of the Emperor of Germany, residing at Südende, near Berlin, Germany, have invented certain new and useful Improvements in a Holder for the Glowes of Tungsten Lamps, (for which I have filed an application in Germany January 30, 1915,) of which the following is a specification.

10 In tungsten lamps, loaded with 0.5-0.8 watt per candle, the so-called half-a-watt lamps, wires of molybdenum or tungsten are made use of for holding the filament wound up to a spiral. On account of the 15 very high temperature, to which the filament is exposed, it becomes necessary to give these holding wires such a thickness that they cannot become too hot. But too strong a heating has the consequence that the holders become 20 soft and get deformed either by their own gravity or by the weight of the glower, the consequence being that in most cases the glow-lamp will become useless. The use of very thin holders is, from such reason, not 25 possible. Now, thick wires have the enormous drawback of withdrawing from the filament very much energy in form of heat. This quantity of energy is not only used to no purpose, it produces also a noxious heating of the whole bulb. This cooling of the 30 filament is to be remarked in the most disagreeable manner with half-a-watt lamps of low candle-power of standard pressures of 110 and 220 volts. Though these lamps radiate 35 a dazzling, white light, their consumption of energy per candle is in most cases far above 0.5 watt.

The present invention avoids this inconvenience and permits also of manufacturing lamps of a low candle power for standard pressures of 110 and 220 volts with a specific consumption of energy of 0.5 watt per candle. It is based upon the observation that tungsten wires having an addition of 1-4% of thorium oxid remain, contrary to wires of 40 tungsten or molybdenum, even in the highest white-heat hard and rigid, whereas at low temperatures they are soft and flexible, so that they may be worked with ease. Consequently such wires constitute an excellent material for making the holders of filaments. They resist to all temperatures to be considered and may be taken so thin that they do not withdraw any appreciable quantity of energy from the filament. They may even be 45 50 55 thinner than the glowing filament itself.

What I claim as my invention and desire to secure by United States Letters Patent is:—

A holder for metallic filament lamps of a 60 low specific consumption of energy, thereby characterized that it consists of tungsten with an addition of 1-4% of thorium oxid, substantially as set forth and for the purpose specified.

In testimony whereof, I affix my signature in the presence of two witnesses.

OTTO SCHALLER.

Witnesses:

HENRY HASPER,  
LILLI FRANK.